

# UNITED STATES PATENT OFFICE.

HANS GOLDSCHMIDT AND OTTO WEIL, OF ESSEN-ON-THE-RUHR, GERMANY, ASSIGNEES  
TO GOLDSCHMIDT THERMIT COMPANY, OF NEW YORK, N. Y., A CORPORATION OF  
NEW YORK.

## PROCESS OF FORMING HIGH-PERCENTAGE TUNGSTEN ALLOYS.

1,235,969.

Specification of Letters Patent.

Patented Aug. 7, 1917.

No Drawing.

Application filed January 20, 1912. Serial No. 672,361.

*To all whom it may concern:*

Be it known that we, HANS GOLDSCHMIDT and OTTO WEIL, subjects of the King of Prussia, German Emperor, and residents of Essen-on-the-Ruhr, in the Province of the Rhine, German Empire, have jointly invented certain new and useful Improvements in Processes of Forming High-Percen-tage Tungsten Alloys, of which the following is an exact specification.

Tungsten alloys of high percentage, which are used for various industrial purposes, more particularly ferro-tungsten were hitherto produced generally in electric furnaces since, as is well known, tungsten can only be fused with difficulty and only at a far higher temperature than chromium and molybdenum for instance. Tungsten alloys produced in electric furnaces always contain carbon so that their use for many industrial purposes is attended with disadvantages.

Attempts have already been made to produce high-grade tungsten alloys by means of so called aluminothermic reactions by causing a mixture for instance of tungstic oxid, ferric oxid and aluminum to react. The output of metal regulus obtained in this way was however, comparatively small, because a large amount of the metal remains in the slag owing to the difficult fusibility of the tungsten.

Considering what was hitherto known about aluminothermic reactions and their applicability to metals of high melting point, it seemed justified to assume that a better output of tungsten alloys of high percentage could only be obtained by adding such substances as raise the temperature of reaction and consequently the energy of reaction. Contrary to the above, experiments have proved that a very good yield of these alloys is obtained by adding indifferent substances to the mixture for the aluminothermic reaction, for example lime or other earths or mixtures of such or similar substances, or fluor-spar which in no way contribute to raising the temperature of reaction and which do not participate in the aluminothermic reaction. In this manner high grade alloys of tungsten particularly with iron, but also with chromium, nickel, molybdenum and other metals can be produced by effecting the aluminothermic reac-

tion of a mixture consisting of tungstic 55 oxid, the oxid of the metal in question, a reducing metal such as aluminum (or a mixture or alloy of several reducing metals) and lime. The quantity of lime added may amount to about a quarter of that of the 60 tungstic oxid used, which appears very surprising and was not to be foreseen.

Instead of adding the lime in this reaction as such it has proved advantageous to use tungstate of calcium as component of the 65 reaction mixture. The tungstate of calcium may be produced artificially or the mineral found in natural state as scheelite ( $CaWO_4$ ) may be used, after being purified in a suitable manner.

This aluminothermic process for obtaining tungsten alloys of high percentage can advantageously be used for incorporating tungsten or tungsten alloys of high percentage into molten metal baths, for instance 75 ferro-tungsten into baths of cast-iron or steel. This incorporation was hitherto made either in form of pulverized metallic tungsten of high percentage (up to 97%) or in the form of ferro-tungsten produced in the 80 electric furnace and containing up to 75-85 per cent. of tungsten. This manner of introduction, however, was highly disadvantageous inasmuch as carbon or oxidation impurities were introduced together with the 85 metallic-tungsten or the ferro-tungsten produced in the electric furnace; further as it was very difficult to alloy these substances with the bath of cast-iron or steel, and finally as one had to reckon a waste of about 90 4-6 per cent. of tungsten. All these disadvantages are avoided by adding to the bath of cast-iron or steel a mixture of ferric-oxid, aluminum tungstic-oxid and, for instance, lime (or instead of the last two substances also tungstate of calcium). The aluminothermic reaction which immediately takes place produces pure ferro-tungsten of high percentage alloying very well and almost without any waste with the cast-iron 100 or steel, the easily fusible slag remaining liquid on the surface of the bath.

Of course the other high grade tungsten alloys mentioned above formed with chromium, nickel, molybdenum and the other 105 metals may also be introduced into molten metal baths in the same manner and with the same success as ferro-tungsten.

What we claim is:

The process of forming alloys containing a high percentage of tungsten which consists in effecting the aluminothermic reaction of a mixture comprising as a component thereof a relatively large quantity of flux, a tungsten compound, the oxid of the alloying metal and a reducing metal.

In witness whereof we have hereunto set our hands in the presence of two witnesses. 10

HANS GOLDSCHMIDT. [L. S.]  
OTTO WEIL. [L. S.]

Witnesses:

CHAS. J. WRIGHT,  
HELEN NUFER.